

## UNITED STATES PATENT OFFICE

2,199,368

## BLUEPRINT COATING

Robert Bowling Barnes, Stamford, and Garnet Philip Ham, Old Greenwich, Conn., assignors to American Cyanamid Company, New York, N. Y., a corporation of Maine

No Drawing. Application June 14, 1939,  
Serial No. 279,056

8 Claims. (Cl. 95—6)

This invention relates to blueprint paper coating and more particularly to improved coating solutions for blueprint paper.

Blueprint paper and similar papers such as, for example, Van Dyke negative paper, require coating of the paper with an aqueous solution of the sensitizing agent. Two of the important characteristics of a good blueprint coating are speed and latitude; that is to say, the exposure time which is required to give sufficiently dark backgrounds for ordinary reproduction and the range of exposure through which tones of adequate color can be obtained. The attempts to increase speed of blueprint papers have resulted in many variations in formulae and some of the fast papers have sacrificed to some extent their latitude.

One of the improved high speed formulae used heretofore is described in the copending application of Garnet Philip Ham, Serial No. 219,599 filed July 16, 1938, now U. S. Patent No. 2,165,166, of July 4, 1939, in which it is shown that amidine compounds when added to a blueprint coating solution have a catalytic effect in that the speed and latitude of the paper are increased as compared to the ordinary blueprint coatings.

In another copending application of Garnet Philip Ham and Robert Bowling Barnes, Serial No. 225,904 filed August 20, 1938, it is shown that treatment of blueprint paper with certain types of wetting agents prior to the application of the blueprint coating solution results in improved blueprint paper as compared to paper not previously coated with the wetting agent.

The blueprint paper produced by using the improved high speed formula described in U. S. Patent No. 2,165,166, of July 4, 1939, and in connection with the method of pre-treatment of the paper with a wetting agent as described in copending application, Serial No. 225,904, is a high quality paper but there is the disadvantage of the necessity for two steps in carrying out the process as it is not feasible to mix the two before using. The fact that it is necessary to apply two individual and separate coatings, namely, the first coating of the wetting agent and the second coating of the sensitized solution, increases the cost of production and somewhat increases the opportunity for lack of uniformity in the final product.

According to the present invention, we have found that sulfonic acid type wetting agents, such as sodium salts of alkyl esters of sulfodicarboxylic acids, when prepared in the form of their

guanidine salts, instead of the sodium salts, can be used in blueprint coating solutions to produce a blueprint paper having improved speed, latitude and greater stability than ordinary blueprint coating.

In general, the class of compounds capable of producing the improved results are the amidine salts of sulfodicarboxylic acid esters as represented by the following type formula:



in which  $R_1$ ,  $R_2$  and  $R_3$  are members of the group consisting of hydrogen, alkyl, hydroxy-alkyl and aryl radicals,  $R_4$  is a dicarboxylic acid ester, and  $X$  is a member of the group consisting of  $R_1$ ,



and



The substituents  $R_1$ ,  $R_2$  and  $R_3$  may be the same or different in various compounds included within the scope of the invention and it should be understood that each symbol is intended to represent any member of the group defined.

An inspection of the above type formula will show that the amidine salts of our invention include salts of guanidine and its derivatives and substitution products, and particularly guanidine itself, guanyl-urea, biguanide, and their alkyl, hydroxyalkyl and aryl substitution products. These compounds are all organic bases, and are sufficiently basic to enable them to form salts with esters of sulfodicarboxylic acids.

Any guanidine base may be used for this purpose, such as guanidine itself, dimethyl or trimethyl guanidine, dibutyl guanidine, mono-, di- or triphenyl guanidine, ditolyl guanidine, or alkoxy substituted guanidines such as mono-, di- or triethanol guanidine and the like. Similarly, such guanyl-urea compounds as guanyl-urea itself, mono- or dimethyl guanyl-urea, diphenyl guanyl-urea, tetraethyl guanyl-urea, and triethanol guanyl-urea are organic bases which will form salts of sulfodicarboxylic acid esters.

The following salts are examples of those that have been found to give excellent results: the guanidine salt of di(methylamyl) ester of sulfosuccinic acid, the guanidine salt of diamyl ester of sulfosuccinic acid, and the guanidine salt of dioctylsulfosuccinic acid.

The reason why these compounds give excellent results in increasing the speed and latitude of the blueprint or sensitized coating has not been definitely determined. However, we believe that 5 there is a two-fold effect: first, the catalytic effect of the guanidine radical promotes greater sensitivity and stability to the coating; and second, the radical producing the wetting effect induces a lower surface tension in the solution 10 which permits greater and more rapid absorption by the paper resulting in a more substantive and uniform coating. These reasons are advanced as a possible partial explanation without limiting the invention thereto.

15 The invention will be described in detail in conjunction with the following specific examples in which these guanidine salts are incorporated in a blueprint formulation without requiring additional components to effect the completion.

## 20 EXAMPLE 1

## Solution A

|                                             |     |     |
|---------------------------------------------|-----|-----|
| Water                                       | ml. | 75  |
| Guanidine salt of dioctylsulfosuccinic acid | g.  | 0.5 |

## Solution B

|                                              |     |       |
|----------------------------------------------|-----|-------|
| Water                                        | ml. | 100   |
| Ferric ammonium oxalate                      | g.  | 24.90 |
| Sodium ferricyanide liquor (21.5 g./100 ml.) | ml. | 12.00 |
| Potassium citrate                            | g.  | 1.00  |
| Citric acid                                  | g.  | 1.00  |

35 Solution A is prepared by heating to about 50° C. to effect rapid dissolution and then cooled to about 25° C. and added to solution B.

40 A sample of ordinary 21 lb.-50% rag stock paper was coated with this sensitized solution and compared to a control paper coated with a solution of the same general formula omitting the guanidine salt of dioctylsulfosuccinic acid. The speed and latitude of the coating were markedly superior to those of the control.

## EXAMPLE 2

45 A blueprint coating was prepared according to the formula of Example 1, except that a stoichiometric amount of potassium ferricyanide crystals was substituted for the sodium ferricyanide. The coating solutions of both Example 1 and 50 Example 2 are greenish brown in color and the dried and sensitized coating is yellow in color.

A blueprint paper was coated using the sen-

sitized formula of Example 2 and compared to a control. The results are the same as Example 1.

## EXAMPLE 3

5 Blueprint paper as described in Example 1 was coated with a sensitized solution prepared according to the formula of Example 1 except the guanidine salt of the di(methylamyl) ester of sulfosuccinic acid was used instead of the 10 guanidine salt of dioctylsulfosuccinic acid.

The results are superior to those of the control but not as good as those of Examples 1 and 2.

## EXAMPLE 4

15 A blueprint coating was prepared as described in Example 2 except the guanidine salt of the di(methylamyl) ester of sulfosuccinic acid was used.

The results are the same as those of Example 3. 20 What we claim is:

1. A blueprint paper coated with a light sensitive blueprint coating composition containing an amidine salt of a sulfodicarboxylic acid ester in an effective amount.

2. A light sensitive blueprint coating composition having as one of the ingredients an amidine salt of a sulfodicarboxylic acid ester in an effective amount.

3. A blueprint paper coated with a light sensitive blueprint coating composition containing a 30 guanidine salt of a sulfosuccinic acid ester in an effective amount.

4. A light sensitive blueprint coating composition having as one of the ingredients a guanidine salt of a sulfosuccinic acid ester in an effective amount.

5. A blueprint paper coated with a light sensitive blueprint coating composition containing the guanidine salt of dioctylsulfosuccinic acid ester.

6. A light sensitive blueprint coating composition having as one of the ingredients the guanidine salt of dioctylsulfosuccinic acid ester.

7. A blueprint paper coated with a light sensitive blueprint coating composition containing the guanidine salt of di(methylamyl) sulfosuccinic acid ester.

8. A light sensitive blueprint coating composition having as one of the ingredients the guanidine salt of di(methylamyl) sulfosuccinic acid ester.

ROBERT BOWLING BARNES.

GARNET PHILIP HAM.